

# United States Patent Office

3,049,392

Patented Aug. 14, 1962

1

3,049,392

## PROCESS FOR DYEING NITROGENOUS MATERIAL WITH SULFONATED COPPER PHTHALOCYANINES

Richard Casty, Kaiserangst, and Heinz Abel, Reinach, Switzerland, assignors to Ciba Limited, Basel, Switzerland

No Drawing. Filed July 29, 1959, Ser. No. 830,189  
Claims priority, application Switzerland Aug. 6, 1958  
9 Claims. (Cl. 8—1)

This invention relates to the dyeing of nitrogenous fibrous material, i.e., to the dyeing of fibers including nitrogen in their chemical constitution.

According to the present invention, there is provided a process for dyeing nitrogenous fibrous material which comprises subjecting said material to treatment in an acid bath containing a sulfonated copper phthalocyanine in the presence of an auxiliary compound which contains at least one basic nitrogen atom to which there is attached at least one radical containing a polyglycol ether chain, wherein the molecule contains at least three groups of the structure



(I)

(preferably  $-\text{CH}_2\text{CH}_2-\text{O}$ -groups) and at least 4 carbon atoms not belonging to such a group, and, after the material has absorbed the required amount of dye, increasing the pH value of the dye bath to above 6.

The process may be applied to any nitrogen-containing fibrous material, for example silk, polyamide fibers consisting of  $\epsilon$ -caprolactam or polyamide fibers consisting of condensates of adipic acid and hexamethylene diamine. However, particular advantages are afforded by the process in the dyeing of wool and of fibrous material containing both fibers of wool and of polyamide.

The sulfonated copper phthalocyanines employed may contain, for example, two, three or four sulfonic acid groups and, if desired, also further substituents such as halogen atoms, more especially chlorine, or sulfonic acid amide groups. Dye mixtures may also be employed, for example sulfonation mixtures whose components differ in the number of sulfonic acid groups, or mixtures of sulfonated copper phthalocyanines with other dyes suitable for dyeing nitrogenous fibers from an acid bath. These latter may be, for example, dyes which contain a mobile halogen atom, i.e. one reactable with the fiber material, preferably a chlorine atom, or dyes consisting substantially of 1:2-chromium or cobalt complex compounds of azo dyes (preferably monoazo dyes) which contain at least two acid water-solubilizing groups in the molecule of the metal complex.

It is characteristic of the present invention that the dyeing is effected in the presence of auxiliary compounds which contain at least one basic nitrogen atom, to which there is attached at least one radical containing a glycol ether chain. This chain contains at least two groupings of the structure I set forth above and may be attached to the nitrogen atom either directly or through a bridge member, for example an alkylene radical, such as an  $n$ -propylene radical. The molecule of the auxiliary compound should contain in total, at least three groups of structure I, preferably groups of the structure:



In addition, the auxiliary compound must contain at least four carbon atoms not belonging to a group of structure I. Thus, it may advantageously contain at least one aliphatic or alicyclic radical comprising at least eight, or preferably twelve, interlinked carbon atoms, or

2

an aromatic radical with an aliphatic side chain, attached to the basic nitrogen atom by an aryl carbon atom.

There are advantageously employed in the present process as nitrogen-containing components of the aforesaid type products of reaction of at least three mols of an  $\alpha,\beta$ -alkylene oxide with 1 mol of an organic compound which contains at least one basic primary or secondary amino group or one basic tertiary amino group and in addition an alcoholic hydroxyl group.

10 As starting materials for the preparation of such products of reaction there may be employed  $\alpha,\beta$ -alkylene oxides such as ethylene oxide, propylene oxide or glycidol. Particularly valuable products are obtained using ethylene oxide.

15 As organic compounds containing at least one primary or secondary amino group, or containing a basic tertiary amino group and in addition an alcoholic hydroxyl group, there may be used amines of the aliphatic and of the aromatic and alicyclic series. Suitable aliphatic amines

20 are monoamines for example diethylamine, butylamine, hexylamine, dodecylamine, cetylamine, oleylamine, octadecylamine, arachidylamine, behenylamine, or mixtures of any of these monoamines. Suitable polyamines are triethylene tetramine and the corresponding N-alkylpoly-

25 amines comprising alkyl radicals of higher molecular weight and containing from 8 to 22 carbon atoms. Basic derivatives of such amines may also be employed, such as esters of hydroxyamines with higher fatty acids, for example triethanolamine cocinic acid esters, or partial

30 amides of polyamines with fatty acids, for example triethylene tetramine monoacylated with cocinic acid. Particularly suitable aromatic amines are amines of the benzene and naphthalene series with alkyl side chains containing, for example, from 8 to 18 carbon atoms.

35 Among alicyclic amines there are preferably employed resin amines such as abietylamine, abiethylmethyamine, the amine mixture corresponding to tall oil (which contains resin amines in addition to higher alkylamines), or hydrogenated abietylamines. In addition, amidines, such as lauric acid or stearic acid amidine, may be employed as starting material.

40 Products suitable for the purpose of the present invention are those obtainable by reaction of 1 mol of an amine as aforesaid with at least 3 mols, for example 3 to 20 mols, of an alkylene oxide, for example:

The reaction product of 1 mol of dodecylamine with about 6 mols of ethylene oxide,

The reaction product of 1 mol of oleylamine, with 6, 8 or 16 mols of ethylene oxide,

The reaction product of 1 mol of stearylamine with 4, 8 or 16 mols of ethylene oxide,

45 The reaction product of monoalkylpropylene diamine, of which the alkyl radical corresponds to the radicals of tallow fatty acids, with 8 mols of ethylene oxide,

The reaction product of monoalkylpropylene diamine, of which the alkyl radical is unbranched and contains from 16 to 18 carbon atoms, and 6 mols of ethylene oxide.

50 The two last mentioned compounds correspond, for example, to the formula:



55 in which R represents an aliphatic hydrocarbon radical preferably unbranched and containing at least 12 and preferably 16 to 22 carbon atoms, m and n represent integers of a value of at most 2, and p, q and r represent

integers, the sum  $p+q+(m-1)(r-1)$  amounting to at least 3 and at most 20 and at least one of the values  $p$ ,  $q$  and  $r-1$  being greater than 1.

Compounds of the formula:



wherein R represents an aliphatic hydrocarbon radical, preferably unbranched and containing at least 12 and preferably from 16 to 20 carbon atoms,  $p$  and  $q$  are integers, and the sum  $p+q$  amounts to at least 3 and preferably to 8 to 16, are preferred compounds for use in the present invention.

The foregoing compounds contain free hydroxy-alkyl groups and there may be used, instead of the free hydroxyl-alkyl compounds, the corresponding esters thereof, e.g. those formed from polybasic acids, for example phosphoric acid or sulfuric acid, or the water-soluble salts of these esters, for example alkali or ammonium or amine salts thereof.

The auxiliary compounds referred to above and employed in the present invention may be produced by methods usual to the production of ethylene oxide addition products, for example by the reaction of the alkylene oxide with the amine at elevated temperature. Preferably, the alkylene oxide is added to the amine only gradually, for example by adding it in gaseous or liquid form to the amine, or introducing it into the latter at a temperature at which the alkylene oxide reacts, for example at 50-200° C. If desired, the operation may be carried out in a closed vessel and under pressure, advantageously at a pressure of from 2 to 10 atmospheres' gauge. If desired, catalysts may be added to the reaction mixture. Such catalysts may with advantage be substances having an alkaline reaction, such as metallic sodium, alkali metal hydroxides, alkali metal carbonates or alkali metal salts of carboxylic acids of low molecular weight.

The products of condensation employed in accordance with the invention are soluble in water or can be readily dispersed therein. The water solubility may if desired be increased by introducing groups which favor water-solubility. Thus, the auxiliary compounds may be formed as quaternary ammonium salts produced by treatment with alkylating agents. Thus, for example the reaction product of oleylamine with 6 to 10 mols of ethylene oxide may be quaternized by treatment with dimethyl sulfate.

In an alternative method of preparation the auxiliary compounds used in the present invention may be obtained by the introduction of polyglycol ether chains with a corresponding number of ether groups into the amines.

The quantities of substances which must be added to the dye baths may vary within relatively wide limits. The quantity of dye naturally depends upon the desired color strength. It is desirable to adapt the quantity of the auxiliary compounds to that of the dye in such manner that the proportion by weight is about 1:8 to 1:2. The quantity of auxiliary compound, however, should be at least 1/4% (calculated on the weight of fiber) even in the case of light dyeing for which less than 1% of dye—also calculated on the fiber weight—is used. Instead of adding the auxiliary compounds and the dyes separately to the dye bath, they may be previously made up as a stable preparation in suitable proportion and this preparation then added.

The dyeing is advantageously carried out in an acetic acid medium, that is to say, in such manner that the dye bath exhibits an acetic acid reaction at least at the beginning of the dyeing. Therefore, there is preferably added to the dye bath at the beginning of the dyeing at least so much acetic acid that the desired pH value is obtained, account having to be taken of the fact that some acid is lost by reaction both with the nitrogenous fibrous

material and by the dyes which are generally present in the form of alkali salts.

As is generally usual in the dyeing of nitrogenous fibrous material, more especially wool, the dyeing operation is preferably carried out at elevated temperature, and most suitably by commencing the actual dyeing process at about 50° to 70° C., heating to boiling temperature and continuing and completing the process at this temperature. After heating to about 90° C., the dye bath may be maintained at this temperature for some time and brought to boiling temperature only when the dye has been substantially completely absorbed by the fiber. In suitable apparatus dyeing may if desired be carried out at temperatures above 100° C., e.g. at about 107° C.

On completion of the actual dyeing operation, the pH value of the bath is raised to a value above 6. Any water-soluble compound having an alkaline reaction is suitable for increasing the pH value, but in order to avoid damage to the fiber, especially in the dyeing of wool, it is desirable to add substances having an alkaline reaction, which raise the pH to a value not exceeding 9. The pH value is with advantage raised to 6.5 to 9. Nitrogenous bases may advantageously be employed for raising the pH value, for example amines such as ethanolamines. In some cases ammonia yields good results and hexamethylene tetramine has proved particularly suitable. Alkali salts of phosphoric acids, more especially dialkali or trialkali orthophosphates or polyphosphates, are also useful for this purpose. A mixture of two or more substances having an alkaline reaction, for example ammonia and hexamethylene tetramine, may be employed.

The after-treatment at the raised pH value need take only a relatively short time, for example about 10 to 30 minutes. It preferably takes place at about the same temperature as that at which the dyeing was effected. For example, the dye bath may be maintained at boiling temperature throughout the after-treatment, or the temperature may be allowed to fall slightly during this after-treatment, for example by supplying no further heat after the increase of the pH value. Finally, the dyed fibrous material may be rinsed and dried as usual with warm and/or cold water.

As a result of the after-treatment at elevated pH value, a part of the dye situated on the fiber returns into the dye bath, but this is dye which is not fixed, or is not properly fixed to the fiber, so that the dyeings obtained by the process of the present invention have better wet fastness properties than the corresponding dyeings produced without subsequent increase of the pH value.

The following examples, in which the parts are by weight, the percentages by weight, and the temperatures, as in the foregoing description, are in degrees centigrade, unless otherwise stated, will serve to illustrate this invention:

#### Example I

A dye bath is formed consisting of 3,000 parts of water, 1 part of copper phthalocyanine trisulfonic acid, 5 parts of 40% acetic acid and 0.5 part of the hereinafter described addition product of oleylamine and ethylene oxide. 100 parts of wool yarn are introduced into the bath at 40° the temperature is raised to 90° during 20 minutes and dyeing is effected at this temperature for about 30 minutes until the dye bath is substantially exhausted. The bath is then brought to boiling temperature and the dyeing is continued at this temperature for 1 hour. There are then added to the bath 2.5 parts of 25% aqueous ammonia solution and 1 part of hexamethylene tetramine. Inadequately fixed dye, which is merely deposited on the surface is thus removed. After further treatment in the boiling bath for 15 minutes, the wool yarn is rinsed, and there is obtained a level, turquoise/blue dyeing having an extremely pure shade and good wet fastness properties.

Without the addition of the auxiliary agent, a much

weaker, very skittery and therefore substantially unusable dyeing is obtained. By the addition of the substances of alkaline reaction towards the end of the dyeing operation, the wet fastnesses (fastness to washing, milling, water and perspiration) are considerably increased.

The ethylene oxide addition product referred to above is prepared as follows:

1 part of finely divided sodium is added to 100 parts of commercial oleylamine and the mixture is heated to 140°. As soon as the ethylene oxide is being rapidly absorbed, the reaction temperature is lowered to 120° to 125° and the introduction of ethylene oxide is continued until 113 parts of ethylene oxide have been absorbed. The reaction product thus obtainable is substantially clearly soluble in water.

#### Example 2

Wool yarn is dyed in accordance with the procedure of Example 1, using copper phthalocyanine-3,3',3'',3'''-tetrasulfonic acid or copper phthalocyanine-3,4',4'',4'''-tetrasulfonic acid instead of copper phthalocyanine tri-sulfonic acid, and the pH value is also increased by the addition of ammonia at the end of the dyeing operation. Blue dyeings are obtained with good wet fastnesses.

Green dyeings are obtained when a mixture of copper phthalocyanine tri- or tetrasulfonic acid and the dye of the formula



is employed.

#### Example 3

Wool yarn is dyed in the manner indicated in Example 1. Instead of the product of reaction of oleylamine and ethylene oxide, however, one of the following products is employed:

- (a) N-alkyl-propylenediamine, of which the alkyl radical corresponds to the radicals of tallow fatty acids, + 8 mols of ethylene oxide,
- (b) N-alkyl-propylene diamine, of which the alkyl radicals are unbranched and saturated and contain from 16 to 18 carbon atoms, + 6 mols of ethylene oxide,
- (c) Mixture of behenylamine and arachidylamine + 8 or 12 mols of ethylene oxide,
- (d) Mixture of the amines obtainable by reduction of the tallow fatty acid amides + 6 to 8 mols of ethylene oxide,
- (e) N-dodecyl-propylenediamine + 6 mols of ethylene oxide,
- (f) Dodecylamine + 3 mols of ethylene oxide,
- (g) Dodecylamine + 3 mols of propylene oxide (24 parts of commercial dodecylamine are heated to 160° in the presence of 0.13 part of finely divided sodium in a current of nitrogen. Gaseous propylene oxide is thereafter introduced until 19.5 parts thereof have been absorbed),
- (h) The sulfuric acid ester obtained by the following procedure: 79 parts of a fatty amine mixture ( $\frac{1}{10}$  mol), consisting of 30% of hexadecylamine, 25% of octadecylamine and 45% of octadecenylamine are reacted with ethylene oxide in the presence of 0.8 part of sodium until 106 parts ( $\frac{2}{10}$  mol) of ethylene oxide have been absorbed. The reaction temperature is initially 140° to 150° and can gradually be lowered to 120° to 125°. There are added to 30.75 parts ( $\frac{1}{20}$  mol) of the re-

sulting ethylene oxide addition product in a stirrer-type vessel at 60° during 15 minutes 5.4 parts of urea, and then during 30 minutes 5.4 parts of sulfamic acid ( $\frac{1}{20}$  mol and 10%), and the mixture is maintained on a boiling water bath for 5 to 6 hours in a current of nitrogen. The product obtained (41 parts) is readily water-soluble and has a neutral reaction.

As indicated in Example 1, the pH value of the dye bath is increased by the addition of ammonia and hexamethylene tetramine, the treatment is continued for 15 minutes in the boiling bath and cold rinsing is then effected. Level, turquoise-blue dyeings of pure color shade and having good wet fastness properties are obtained.

#### Example 4

The procedure of the preceding examples is followed, but there is added to the dye bath, to increase the pH value, instead of ammonia and hexamethylene tetramine, ammonia alone, sodium bicarbonate, sodium triphosphate or triethanolamine. The dyeings thus after-treated are also distinguished by good wet fastness properties.

#### Example 5

25 A mixed fabric or blended yarn consisting of wool and polyamide fibers in equal proportions, is dyed in accordance with the procedure of one of Examples 1 to 3, the

pH value also being increased in the manner indicated. Level dyeings are obtained.

What is claimed is:

1. A process for dyeing nitrogenous fibrous material, which comprises subjecting said material to treatment in an acid bath containing a sulfonated copper phthalocyanine in the presence of an auxiliary compound of the formula



50 in which R represents an aliphatic hydrocarbon radical containing at least 12 carbon atoms, in each of the groupings  $-\text{CHX}-\text{CHX}-\text{O}-$  at least one of the two X's represents a hydrogen atom and any X not representing hydrogen stands for a methyl group, m and n are integers of at the most 2, and p, q and r are integers, the sum  $p+q+(m-1)(r-1)$  amounting to at least 3 and to at most 20, and, after the material has absorbed the required amount of dye, increasing the pH value of the dyebath to above 6.

60 2. A process for dyeing wool which comprises subjecting the wool to treatment in an acid bath containing a sulfonated copper phthalocyanine in the presence of an auxiliary compound of the formula



in which R represents an aliphatic hydrocarbon radical containing at least 12 carbon atoms, in each of the groupings  $-\text{CH}_2-\text{CH}_2-\text{O}-$  at least one of the two X's represent a hydrogen atom and any X not representing hydrogen stands for a methyl group, m and n are integers of at the most 2, and p, q and r are integers, the sum  $p+q+(m-1)(r-1)$  amounting to at least 3 and to at most 20, and, after the material has absorbed the required amount of dye, increasing the pH value of the dyebath to above 6.

3. A process for dyeing wool which comprises subjecting the wool to treatment in an acid bath containing a sulfonated copper phthalocyanine in the presence of an auxiliary compound of the formula



in which R represents an aliphatic hydrocarbon radical containing at least 12 and at the most 22 carbon atoms, m and n are integers of at most 2, and p, q and r are integers, the sum  $p+q+(m-1)(r-1)$  amounting to at least 3 and to at most 20, and, after the material has absorbed the required amount of dye, increasing the pH value of the dyebath to above 6.

4. A process for dyeing wool which comprises subjecting the wool to treatment in an acid bath containing a sulfonated copper phthalocyanine in the presence of an auxiliary compound of the formula



in which R represents an aliphatic hydrocarbon radical containing 12 to 20 carbon atoms, and p and q are integers, the sum  $p+q$  amounting to at least 3 and to at the most 22, and, after the material has absorbed the required amount of dye, increasing the pH value of the dyebath to above 6.

5. A process for dyeing wool which comprises subjecting the wool to treatment in an acid bath containing a copper phthalocyanine trisulfonic acid in the presence of an auxiliary compound of the formula



in which R represents an aliphatic hydrocarbon radical containing at least 12 carbon atoms, in each of the groupings  $-\text{CH}_2-\text{CH}_2-\text{O}-$  at least one of the two X's represent a hydrogen atom and any X not representing hydrogen stands for a methyl group, m and n are integers of at the most 2, and p, q and r are integers, the sum  $p+q+(m-1)(r-1)$  amounting to at least 3 and to at most 20, and, after the material has absorbed the required

amount of dye, increasing the pH value of the dyebath to above 6.

6. A process for dyeing wool which comprises subjecting the wool to treatment in an acid bath containing a copper phthalocyanine tetrasulfonic acid in the presence of an auxiliary compound of the formula



15 in which R represents an aliphatic hydrocarbon radical containing at least 12 carbon atoms, in each of the groupings  $-\text{CH}_2-\text{CH}_2-\text{O}-$  at least one of the two X's represents a hydrogen atom and any X not representing hydrogen stands for a methyl group, m and n are integers of at the most 2, and p, q and r are integers, the sum  $p+q+(m-1)(r-1)$  amounting to at least 3 and to at most 20, and, after the material has absorbed the required amount of dye, increasing the pH value of the dyebath to above 6.

20 7. A process for dyeing wool which comprises subjecting the wool to treatment in an acid bath containing a sulfonated copper phthalocyanine in the presence of an ethylene oxide addition product obtained from one molecular proportion of oleylamine and about 7 molecular proportions of ethylene oxide, and, after the material has absorbed the required amount of dye, increasing the pH value of the dyebath to above 6.

8. A process for dyeing wool which comprises subjecting the wool to treatment in an acid bath containing a copper phthalocyanine trisulfonic acid in the presence of an ethylene oxide addition product obtained from one molecular proportion of oleylamine and about 7 molecular proportions of ethylene oxide, and, after the material has absorbed the required amount of dye, increasing the pH value of the dyebath to above 6.

40 9. A process for dyeing wool which comprises subjecting the wool to treatment in an acid bath containing a copper phthalocyanine tetrasulfonic acid in the presence of an ethylene oxide addition product obtained from one molecular proportion of oleylamine and about 7 molecular proportions of ethylene oxide, and, after the material has absorbed the required amount of dye, increasing the pH value of the dyebath to above 6.

#### References Cited in the file of this patent

#### UNITED STATES PATENTS

|           |             |       |               |
|-----------|-------------|-------|---------------|
| 1,970,578 | Schoeller   | ----- | Aug. 21, 1934 |
| 2,484,300 | Mayhew      | ----- | Oct. 11, 1949 |
| 2,681,845 | Luttinghaus | ----- | June 22, 1954 |
| 2,761,868 | Lacey       | ----- | Sept. 4, 1956 |
| 2,914,538 | Randall     | ----- | Nov. 24, 1959 |
| 2,967,755 | Kelier      | ----- | Jan. 10, 1961 |

#### OTHER REFERENCES

- 60 Vankataraman: "Synthetic Dyes," vol. II, pub. 1952 by Academic Press Inc., N.Y.C., pages 1128-1135.

UNITED STATES PATENT OFFICE  
CERTIFICATE OF CORRECTION

Patent No. 3,049,392

August 14, 1962

Richard Casty et al.

It is hereby certified that error appears in the above numbered patent requiring correction and that the said Letters Patent should read as corrected below.

Column 5, lines 28 to 38, for that portion of the formula reading



column 6, line 20, for "of" read -- or --.

Signed and sealed this 3rd day of September 1963.

(SEAL)

Attest:

ERNEST W. SWIDER

Attesting Officer

DAVID L. LADD

Commissioner of Patents